# EUROPEAN PATENT SPECIFICATION

(11) **EP 0 488 744 B1**
(45) Date of publication and mention of the grant of the patent: **17.07.1996**
(21) Application number: 91311035.9
(22) Date of filing: 28.11.1991
(51) Int. Cl.: G03G 9/087, G03G 9/097

(54) **Electrophotographic toner for negative charging**
Elektrophotographischer Toner für Negativaufladung
Toneur électrophotographique pour charger négativement

(30) Priority: 28.11.1990 JP 328363/90
(43) Date of publication of application: 03.06.1992
(73) Proprietor: MITA INDUSTRIAL CO., LTD., Osaka 540 (JP)
(72) Inventor: Tsubota, Noriaki, Himeji-shi, Hyogo-ken (JP); Kubo, Masahiko, Yao-shi, Osaka-fu (JP); Fuji, Kazuo, Higashi-osaka-shi, Osaka-fu (JP); Watanabe, Akihiro, Kita-katsuragi-gun, Nara-ken (JP); Kuramae, Yoshihisa, Hirakata-shi, Osaka-fu (JP)
(74) Representative: Cresswell, Thomas Anthony

(56) References cited:
- EP-A- 0 203 818
- EP-A- 0 276 963
- EP-A- 0 284 000
- EP-A- 0 330 287
- EP-A- 0 430 700
- PATENT ABSTRACTS OF JAPAN vol. 14, no. 167 (P-1031)(4110) 30 March 1990; & JP-A-2 022 670 ( RICOH ) 25 January 1990
- PATENT ABSTRACTS OF JAPAN Vol. 10, no. 305 (P-507)(2361) 17 October 1986; & JP-A- 61 118 761 ( FUJITSU LDT ) 6 June 1986

## Description

### Background of the Invention

### (1) Field of the Invention

The present invention relates to an electrophotographic toner for negative charging. More particularly, the present invention relates to an electrophotographic toner for negative charging, which is capable of forming a high-density image without scattering of the toner.

### (2) Description of the Related Art

In commercial electrophotographic reproduction or electrophotographic printing, in order to reduce the amount of ozone generated at the charging step, there is ordinarily adopted a process in which an electrostatic image positively charged is formed, and therefore, a toner for negative charging is widely used as the developing toner for developing this electrostatic image.

Recently, development of a laser beam printer or a digital copying machine has advanced, and in this image-forming apparatus, there is adopted an operation of writing a latent image into an organic photosensitive material of the negative charging type by a laser and performing reversal development by a toner for negative charging, and a high quality is also required for the toner negative charging.

The developing toner is generally formed by pulverizing a resin composition comprising a fixing resin, a colorant and a charge-controlling agent as indispensable components into an average particle size of 5 to 15 µm. Naturally, a charge-controlling agent exerting a negative charge-controlling action at the frictional charging is used in case of a toner for negative charging.

In the conventional toner charge-controlling process, the average value of the charge quantity as the entire toner is controlled according to the kind of the charge-controlling agent or the amount added of the charge-controlling agent. However, even if the average value of the charge quantity as the entire toner can be controlled, it is very difficult to strictly control the distribution of the charge quantity in toner particles.

It is known that a plurality of charge-controlling agents having charging performances reverse to each other are incorporated in toner particles. For example, Japanese Unexamined Patent Publication No. 54-34243 discloses a developer for developing an electrostatically charged image, comprising a toner and a carrier, in which the toner is a toner for negative charging, which comprises a dye positively charged by friction with the carrier.

Furthermore, Japanese Unexamined Patent Publication No. 57-196264 discloses an electrically insulating magnetic one-component developer comprising an electrically insulating fixing medium and, dispersed in the fixing medium, a magnetic material powder and a charge-controlling agent, in which the charge-controlling agent comprises a negative or positive charge-controlling agent and a charge-controlling agent having a reverse polarity at a weight ratio of from 1/0.05 to 1/1.5.

EP-A-0,276,963 discloses a negatively chargeable toner for use in dry electrophotography comprising a resinous binder which is a copolymer of styrene and an alkyl (meth)acrylate and a styrene-acrylamide copolymer containing a sulphonic acid group.

JP-A-2-22670 discloses a toner comprising both negative and positive charge-controlling agents to stabilize potential acceptance without being affected by variance of environmental conditions.

In the conventional toner for negative charging, even though the average value of the charge quantity can be maintained at a satisfactory level by adjusting the kind or amount added of the charge-controlling agent, a disadvantage of considerable broadening of the distribution of the charge quantity cannot be eliminated. Namely, a highly charged toner having a much larger charge quantity than the average value, which is not consumed for the development, is inevitably generated at a certain frequency (distribution quantity). Furthermore, a lowly charged toner having a much smaller charge quantity than the average value and causing scattering of the toner is generated at a certain frequency.

Particles of the former highly charged toner are electrically strongly attracted to surfaces of the carrier particles and are present in a hardly separable state, and they extraordinarily inhibit frictional chargeability performances of the carrier particles. Accordingly, even in case of a toner causing no particular problem at the initial stage of the development, with the lapse of the developing time, the proportion of the uncharged or lowly charged toner increases, and such troubles as scattering of the toner, fogging and reduction of the image density are caused.

In the above-mentioned prior art process in which a charge-controlling agent for negative charging is combined with a positively chargeable dye (charge-controlling agent), there can be attained an advantage that the distribution of the charge quantity can be considerably freely shifted to the high charge quantity side or the low charge quantity side, but this process is still insufficient for sharpening the distribution of the charge quantity of the toner and controlling formation of a highly charged toner or a lowly charged toner completely or to a level that can be neglected.

### Summery of the Invention

It is a primary object of the present invention to overcome the above-mentioned defects of the conventional toner for negative charging and provide a toner for negative charging, in which the charge quantity of the toner can be preferably adjusted, the average value of the charge quantity of the toner is arranged within a range optimum for prevention of scattering of the toner and reduction of the image density, the distribution of the charge quantity of the toner is sharp, and there are hardly present a highly charged toner not used for the development and a lowly charged toner causing scattering of the toner.

Another object of the present invention is to provide a toner for negative charging, in which the distribution of the charge quantity of the toner is sharp, rise of the charge is quick at the time of charging, and at the long-time operation the charging characteristics are hardly degraded.

In accordance with the present invention, there is provided an electrophotographic toner for negative charging, comprising a fixing resin, a colorant, a charge-controlling agent for negative charging which is a copolymer of an acrylamide monomer of formula (1)

CH₂ = CX¹ - CONH - X² - SO₃H (1)

wherein X¹ is hydrogen or methyl and X² is a divalent
hydrocarbon group having 1 to 6 carbon atoms, and a vinylic monomer, and a charge-controlling assistant which is a positive charge-controlling substance which is incompatible with the fixing resin and is dispersed therein, and which charge-controlling assistant is a compound of formula (II)
wherein one or two of the groups R are alkyl or alkenyl having at least 8 carbon atoms and the other groups R are alkyl of up to 4 carbon atoms or benzyl and A⁻ is an oxyacid anion.

It is preferred that the charge-controlling agent (A) and the charge-controlling assistant (B) be present at an (A)/(B) weight ratio of from 1/0.05 to 1/1, especially from 1/0.1 to 1/0.7, and it also is preferred that the charge-controlling agent and charge-controlling assistant be used in a total amount of 0.5 to 5 parts by weight, especially 2 to 4 parts by weight, per 100 parts by weight of the fixing resin.

### Brief Description of the Drawings

Fig. 1 is a diagram illustrating the distribution of the charge quantity of the toner of the present invention (Example 1).

Fig. 2 is a diagram illustrating the distribution of the charge quantity of the toner for negative charging (Comparative Example 1), in which the positive charge-controlling substance is not incorporated.

Fig. 3 is a diagram illustrating the distribution of the charge quantity of a toner in which a charge-controlling agent for negative charging and a positively chargeable dye compatible with a fixing resin are incorporated in combination.

Fig. 4 is a diagram illustrating an apparatus for measuring the charge quantity of the toner.

Fig. 5 is a diagram illustrating the distribution of the charge quantity after formation of 50,000 copies, observed with respect to the toner of Example 1.

Fig. 6 is a diagram illustrating the distribution (curve A) of the initial charge quantity and the distribution (curve B) of the charge quantity after formation of 5,000 copies, observed with respect to the toner of Comparative Example 3.

Fig. 7 is a diagram illustrating the distribution (curve A) of the initial charge quantity and the distribution (curve B) of the charge quantity after formation of 50,000 copies, observed with respect to the toner of Example 3.

Fig. 8 is a diagram illustrating the distribution (curve A) of the initial charge quantity and the distribution (curve B) of the charge quantity after formation of 50,000 copies, observed with respect to the toner of Example 5.

Fig. 9 is a diagram illustrating the distribution (curve A) of the initial charge quantity and the distribution (curve B) of the charge quantity after formation of 50,000 copies, observed with respect to the toner of Example 7.

### Detailed Description of the Invention

The present invention is based on the finding that if a positive charge-controlling substance incompatible with a fixing resin but dispersible therein is combined as the charge-controlling assistant with a charge-controlling agent for negative charging, instead of a positively chargeable dye compatible with the fixing resin, conventionally used, the distribution of the charge quantity can be made conspicuously sharper than in the conventional toner, with the result that generation of a highly charged toner not used for the development or a lowly charged toner causing scattering of the toner can be effectively controlled.

These effects of the present invention can be readily understood from Figs. 1 through 3 showing the distributions of charge quantities of toners.

The distributions of charge quantities shown in Figs. 1 through 3 are determined by using a charge quantity-measuring apparatus shown in Fig. 4 according to the following method.

### Measurement of Distribution of Charge Quantity

The charge quantity-measuring apparatus shown in Fig. 4 comprises a separating portion 2 arranged in a cylindrical housing 1 to separate a toner from a developer, a measuring portion 3 for measuring the distribution of the charge quantity of the separated toner, and a sucking device 11 such as an air pump.

The separating portion 2 is separated from the measuring portion 3 by a partition plate 7. A circulating hole 1a for introducing air into the housing 1 is formed on the side wall of the housing 1 slightly below the partition plate 7. An air-rectifying filter 8 is arranged slightly below the circulating hole 1a.

In the separating portion 2, compressed air is blown by an air needle 5 to a developer maintained on a magnet 4, whereby only the light toner is blown up and scattered while leaving a carrier attracted magnetically to the magnet 4.

A funnel 6 supported by the partition plate 7 is arranged between the separating portion 2 and the measuring portion 3. A receiving opening 6d on the top end of the funnel 6 projects above the partition plate 7, and a dent 6a on the lower end pierces through the filter 8 and is exposed to the side of the measuring portion 3.

In the measuring portion 3, by applying a direct current power R to a pair of electrode rods 9a and 9b embedded in the side wall of the housing 1, a horizontal parallel electric field is formed between the electrode rods 9a and 9b. Reference numeral 10 represents a filter.

The sucking device 11 forms a main air current flowing from the outside of the housing 1 to the measuring portion 3 through the circulating hole 1a and the rectifying filter 8 and also forms an air current for sucking the toner into the funnel 6 above the funnel 6.

In the above-mentioned charge quantity-measuring apparatus, the toner particles separated by the separating portion 2, collected by the funnel 6 and introduced into the measuring portion are vertically dropped while being carried by the air current formed by the sucking device 11 and are allowed to fall on the filter 10 through between the electrode rods 9a and 9b. Since the toner particles fall down in the horizontal parallel electric field between the electrode rods 9a and 9b under Coulomb force H corresponding to the charge quantity in the horizontal direction and gravity V in the vertical direction. Accordingly, the toner particles are dispersed on the filter 10 at a position corresponding to the mass or charge quantity thereof. Then, from the distribution of falling positions of the toner particles, the distribution of the charge quantity of the toner is calculated by an image treatment.

The charge quantity distributions curves shown in Figs. 1, 2 and 3 are those determined according to the above-mentioned method.

In case of toner A where a controlling agent for negative charging alone is used (toner of Comparative Example 1), as shown in Fig. 2, a highly charged toner in area a is present in a large quantity, and a reversely charged toner or an uncharged toner in zone d is contained in a considerable proportion. In case of toner B of the prior art where a positively chargeable dye is combined with a controlling agent for negative charging (toner of Comparative Example 2), as shown in Fig. 3, the average value of the charge quantity can be shifted to a low charge quantity side but the distribution width is not substantially changed from that of toner A, the amount of the highly charged toner is reduced but the highly charged toner is still present, and the proportion of the reversely charged toner or uncharged toner in area d increases. In contrast, in case of toner C of the present invention where a controlling agent for negative charging is combined with a positive charge-controlling assistant in compatible with a fixing resin (toner of Example 1), the quantity of the toner present in appropriate charging areas b and c increases and the width of the distribution of the charge quantity is drastically narrowed, and the quantity of the highly charged toner in area a or the reversely charged or uncharged toner in area d is reduced (is not present in this case).

By using the foregoing toners A, B and C, copying for obtaining 5,000 prints is continuously carried out in a remodelled machine (the developing process is changed to the reversal developing process) of Laser Beam Printer LPX-1 (Registered Trade Mark in one or more designated states) (supplied by Mita Industrial Co.), and the image density (ID), the fog density (FD) of the image and scattering of the toner in the periphery of the developing device are examined. The obtained results are shown in Table 1.

**Table 1**

| Toner | Image Density (ID) | Fog Density (FD) of Image | Toner Scattering (FD) |
|---|---|---|---|
| A | 1.25 - 1.32 | 0.001 - 0.009 | conspicuous |
| B | 1.30 - 2.45 | 0.005 - 0.010 | very conspicuous |
| C | 1.30 - 1.32 | below 0.001 | not observed |

From Figs. 1 through 3 and Table 1, it is understood that the toner of the present invention has such preferred charging characteristics that variation of the image density, formation of fogging of the image and scattering of the toner can be controlled.

In the toner of the present invention, not only at the initial stage of the development, but also when the development is continued for a long time, variation of the image density, occurrence of fogging and scattering of the toner are not caused and a high effect of preventing the deterioration can be attained.

The fact that by using a charge-controlling assistant for positive charging, which is in compatible with the fixing resin, in the toner of the present invention, the distribution of the charge quantity can be sharpened was found as a phenomenon as the result of many experiments. The reason has not been elucidated, but since a positively chargeable dye compatible with the fixing resin has no effect of sharpening the distribution, it is estimated that the dispersion structure in which in a matrix having the controlling agent for negative charging dissolved or dispersed therein, the positively chargeable substance is dispersed in a larger macro particle size will exert a function of reducing numbers of the highly charged toner and the negatively charged toner. In general, one of serious defects of the combination of the positive charge-controlling substance as the assistant with the negative charge-controlling agent is that when a developer comprising this toner and a carrier is stirred in the developing device, rising of the charge is delayed, even though the charge of the toner particles is finally controlled to a negative value. In contrast, in the toner having the composition and dispersion structure specified in the present invention, when the developer is stirred to initiate stirring, rising of the charge is as quick as in case of the negatively chargeable toner comprising a negative charge-controlling agent alone. This is another advantage attained by the present invention.

It is also important to use a copolymer composed of an acrylamide-type monomer of general formula (1) and a vinyl-type monomer. This copolymer dissolves in the form of a transpatent or pale-colored transparent state in the fixing resin and gives a very stable negative charging properties. The toner of this invention as shown in Examples, shows almost the same charging property as in the initial state even when a copying step was repeated many times. The use of such a copolymer as a negative charge controlling agent is one example for this reason.

The negatively chargeable toner of the present invention can be effectively used not only as a toner for forming an ordinary single-color image but also as a toner for forming a so-called full-color image. For example, a full-color image can be formed by lapping a cyan toner, a yellow toner and a magenta toner, but it sometimes happens that the charging characteristics of the respective color toners are changed by a mechanical impact force or heat generated by the stirring operation in the developing device. More specifically, even if the distribution of the charge quantity of each color toner is sharp, it is difficult to maintain this state while continuing the copying operation. Furthermore, if the charging characteristics of each color toner are changed, development of the color toner is not effectively attained, and a desired full-color image can hardly be reproduced. According to the present invention, a sharp distribution of the charge quantity can be effectively maintained over a long period, and the above problem in formation of a full-color image can be effectively eliminated.

### Charge-Controlling Assistant

The positive charge-controlling substance used as the charge-controlling assistant in the present invention is a quaternary ammonium salt incompatible with the fixing resin but dispersible therein and has a charge-controlling action of a polarity reverse to that of the charge-controlling agent for negative charging.

As the quaternary ammonium salt, there is preferably used a compound represented by the following formula: (2): wherein at least one of groups R represents a long-chain alkyl or long-chain alkenyl group having at least 8 carbon toms, especially 8 to 22 carbon atoms, other groups R represent a lower alkyl group, a benzyl group, a long chain alkyl group of a long-chain alkyl group, with the proviso that at least 2 of these groups R represent a lower alkyl group having up to 4 carbon atoms or a benzyl group, and A represents an oxyacid anion.

As the oxyacid anion, there can be mentioned anions of oxyacids such as orthophosphoric acid and pyrophosphoric acid, molybdic acid, tungstic acid, antimonic acid and bismuthic acid. These quaternary ammonium salts are especially suitable for sharpening the distribution of the charge quantity without delaying rising of charging of the toner.

### Charge-Controlling Agent

The negative electric charging agent to be used in combination with the electric charging assistant is a copolymer of an acrylamide-type monomer of

CH₂ = CX¹ - CO-NH - X² - SO₃H (1)

and a vinyl-type monomer.

In formula (1) showing the acrylamide-type monomer, X¹ is a hydrogen atom or a methyl group, preferably a hydrogen atom, X² is a divalent hydrocarbon group having 1 to 6 carbon atoms, such as an alkylene group. Specific examples of the acrylamide-type monomer include 3-acrylamide-3-methylbutylsulfonic acid, 2-acrylamide-2-methylbutylsulfonic acid, and 2-acrylamide-2-butylpropanesulfonic acid. Most preferred is 2-acrylamide-2-methylsulfonic acid.

As the vinyl-type monomer, various known monomers may be used. Preferably, styrene and α-methyl-styrene. Most preferably, styrene may be used.

In the above copolymer, the content of the acrylamide-type copolymer is preferably 2 to 20 % by weight, the negative charging property tends to be lost. Furthermore, the weight average molecular weight (Mw) of the copolymer is preferably 2,000 and 15,000.

In the present invention, the charge-controlling agent and the charge-controlling assistant are preferably used at a weight ratio of from 1/0.005 to 1/1, especially from 1/0.1 to 1/0.7. It is preferred that the combination of the charge-controlling agent and charge-controlling assistant be present in an amount of 1 to 5 parts by weight, especially 2 to 4 parts by weight, per 100 parts by weight of the fixing resin.

### Fixing Resin

A known resin which is not compatible with the charge-controlling assistant but is capable of dispersing the charge-controlling assistant therein is used as the fixing resin. Since the fixing resin negatively charges the toner, it is preferred that the fixing resin should have a tendency to be negatively charged. For example, a styrene resin, an acrylic resin, a styrene-acrylic resin and a polyester resin are generally used.

As the styrene monomer constituting the fixing resin, there can be mentioned monomers represented by the following formula: wherein R₁ represents a hydrogen atoms, a lower alkyl group (having up to 4 carbon atoms) or a halogen atom, R₂ represents a hydrogen atom or a substituent such as a lower alkyl group or a halogen atom,
such as styrene, vinyltoluene, α-methylstyrene, α-chlorostyrene and vinylxylene, and vinylnaphthalene. Of these monomers, styrene is preferably used.

As the acrylic monomer, there can be mentioned monomers represented by the following formula: wherein R₃ represents a hydrogen atom or a lower alkyl group, and R₄ represents a hydrogen atom or a substituted or unsubstituted alkyl group having up to 18 carbon atoms,
such as ethyl acrylate, methyl methacrylate, butyl acrylate, butyl methacrylate, 2-ethylhexyl acrylate, 2-ethylhexyl methacrylate, acrylic acid and methacrylic acid. As the acrylic monomer, there can be used other ethylenically unsaturated carboxylic acids and anhydrides thereof, such as maleic anhydride, crotonic acid and itaconic acid.

A styrene acrylic copolymer resin is one of preferred fixing resins, and the weight ratio A/B of the styrene monomer (A) to the acrylic monomer (B) is preferably from 50/50 to 90/10, especially preferably from 60/40 to 85/15. Preferably, the acid value of the resin used is 0 to 25. From the viewpoint of the fixing property, it is preferred that the resin should have a class transition temperature (Tg) of 50 to 75°C.

Generally, it may be obtained preferably as a polyester resin obtained by polycondensing a diol component represented by the formula: wherein R is an ethylene group or propylene group, and m or n is a positive integer,
with a polycarboxylic acid or acid anhydride as an acid component or its derivative.

Examples of the diol component include polyoxypropylene-2,2-bis(4-hydroxyphentl) propane, polyoxyethylene-2,2-bis(4-hydroxyphentl)propane, and polyoxypropylene-polyoxyethylene-2,2-bis(4-hydroxyphenyl) propane.

Examples of the carboxylic acid are maleic acid, fumaric acid, mesaconic acid, citraconic acid, taconic acid, glutaconic acid, phthalic acid, isophthalic acid, terephthalic acid, cyclohexanedicarboxylic acid, succinic acid, adipic acid, sebacid acid, malonic acid, 1,2,4-benzenetricarboxylic acid, 1,2,5-benzenetricarboxylic acid, 1,2,4-cyclohexanetricarboxylic acid, 2,5,7-naphthalenetricarboxylic acid, 1,2,4-naphthalenetricarboxylic acid, 1,2,5-hexanetricarboxylic acid, 1,2,4-butanetricarboxylic acid, 1,3-dicarboxy-2-methylcarboxypropen, 1,3-dicarboxylic-2-methyl-2-methylcarboxy propane tetra(methylene carboxy)methane, 1,2,7,8-octanetetracatboxylic acid, enball trimer and anhydrides of these.

This polyester resin may be produced by polycondensing the diol component with the polycarboxylic acid component. It the reaction, other diol components such as ethylene glycol and bisphenol A in addition to 10 mole% of may be concurrently used etherified bisphenols A of the above formula.

### Colorant

As the colorant to be incorporated into the binder resin, there can be used at least one member selected from the group consisting of inorganic and organic pigments and dyes, for example, carbon blacks such as furnace black and channel black, iron blacks such as triiron tetroxide, rutile titanium dioxide, anatase titanium dioxide, Phthalocyanine Blue, Phthalocyanine Green, cadmium yellow, molybdenum orange, Pyrazolone Red and Fast Violet B.

In the case where the toner of the present invention is used as the yellow toner for full-color development, for example, there are preferably used benzidine pigments such as C.I. Pigment Yellow 13 (Benzidine Yellow GR) (Registered Trade Mark in one or more designated states), C.I Pigment Yellow 14 (Vulcan Fast Yellow G) (Registered Trade Mark in one or more designated states), C.I. Pigment Yellow 17 (Registered Trade Mark in one or more designated states), C.I. Pigment Yellow 55 (Registered Trade Mark in one or more designated states), C.I. Pigment Yellow 12 (Registered Trade Mark in one or more designated states) and C.I. Pigment Yellow 83 (Registered Trade Mark in one or more designated states). In this case, a yellow colorant such as chrome yellow, titanium yellow or quinoline yellow lake can be used in addition to the benzidine pigment according to need.

In the case where the toner of the present invention is used as the magenta toner full-color development, quinacridone pigments such as C.I. Pigment Red 122 (Quinacridone Magneta) (Registered Trade Mark in one or more designated states), C.I. Pigment Red 192 (Registered Trade Mark in one or more designated states), C.I. Pigment Red 209 (Registered Trade Mark in one or more designated states) and C.I. Pigment Violet 19 (Quinacridone Violet) (Registered Trade Mark in one or more designated states) are preferably used.

In the case where the toner of the present invention is used as the cyan toner for full-color development, copper phthalocyanine pigments such as C.I. Pigment Blue 15 (Phthalocyanine Blue) (Registered Trade Mark in one or more designated states), C.I. Pigment 16 (Heliogen Blue G) (Registered Trade Mark in one or more designated states) and C.I. Pigment Blue 17 (Fast Sky Blue) (Registered Trade Mark in one or more designated states) are preferably used.

the colorant is generally used in an amount of 2 to 15 parts by weight, preferably 3 to 10 parts by weight, per 100 parts by weight of the resin.

### Toner

The particle size of toner particles is such that the volume-based median diameter measured by a Coulter Counter is 5 to 15 um, especially 7 to 12 um. The particles can have an indeterminate shape formed by melt-mixing and pulverization or a spherical shape formed by dispersion or suspension polymerization.

The toner of the present invention is combined with a known magnetic carrier and used as a two-component magnetic developer to exert excellent charging characteristics.

As the magnetic carrier, there can be used a ferrite carrier and an iron powder carrier. The carrier can be used in an uncoated stated or resin-coated stated. In general, a ferrite carrier is preferably used.

As the ferrite, there have been used sintered ferrite particles composed of at least one member selected from the group consisting of zinc iron oxide (ZnFe₂O₄), Yttrium iron oxide (Y₃Fe₅O₁₂), cadmium iron oxide (CdFe₂O₄), gadolinium iron oxide (Gd₃Fe₅O₁₂), copper iron oxide (CuFe₂O₄), lead iron oxide (PbFe₁₂O₁₉), nickel iron oxide (NiFe₂O₄), neodium iron oxide (NdFeO₃), barium iron oxide (BaFe₁₂O₁₉), magnesium iron oxide (MgFe₂O₄), manganes iron oxide (MnFe₂O₄) and lanthanum iron oxide (LaFeO₃). Especially, soft ferrites containing at least one member, preferably at least two members, selected from the group consisting of Cu, Zn, Mg, Mn and Ni, for example, a copper/zinc/magnesium ferrite, can be used.

As the coating resin for magnetic carriers, there are known an acrylic resin, a styrene resin, a silicone resin, a fluorine resin and an amino-modified resin. A resin that controls indirectly the toner charge to a negative level by controlling the charge of the resin-coated magnetic carrier to a positive level is preferably used. Of course, in the present invention, even if this carrier-coating resin is not present, control of the charge can be accomplished effectively and assuredly.

It is preferred that the saturation magnetization of the carrier be 40 to 75 emu/g, especially 45 to 70 emug. A ferrite carrier satisfying the above requirement, especially a ferrite carrier having a spherical shape, is preferably used. It is preferred that the particle size of the ferrite carrier be 20 to 140 µm, especially 50 to 100 µm.

The mixing ratio of the toner and the magnetic carrier depends on the physical properties of the toner and the magnetic carrier, but it is preferred that the mixing weight ratio be in the range of from 1/99 to 10/90, especially from 2/98 to 5/95.

It also is preferred that the resistivity of the developer as a whole be 5 x 10⁹ to 5 x 10¹² Ω -cm, especially 5 x 10⁹ to 5 x 10¹¹ Ω-cm.

At the development of an electrostatic image, the above-mentioned toner and magnetic carrier are mixed, a magnetic brush having a predetermined length is formed on a developing sleeve having a magnet roll arranged therein, and the magnetic brush is brought into sliding contact with a photosensitive material having the electrostatic image, or the magnetic brush is brought into close proximity to the electrostatic image-holding photosensitive material in a field to which a vibrating electric field is applied.

### Examples

The present invention will now be described in detail with reference to the following examples that by no means limit the scope of the invention.

### Example 1

By a twin-screw kneader, 100 parts by weight of a styrene/acrylic copolymer as the fixing resin, 5 parts by weight of carbon black as the colorant, 1.5 parts by weight of low-molecular-weight polypropylene as the offset-preventing agent, 2 parts by weight of a copolymer of styrene and 2-acrylamide-2-methylpropane sulfonic acid (styrene content; 91%, Mw: 8000) as the charge-controlling agent for negative charging and 0.5 part by weight of a quaternary ammonium salt represented by the following formula: as the charge-controlling assistant incompatible with the styrene/acrylic copolymer were melt-kneaded, and the melt-kneaded mixture was cooled, pulverized and sieved to obtain a toner having an average particle size of 11 um. The toner was mixed and stirred with a resin-coated ferrite carrier having an average particle size of 85 µm at a toner concentration of 4.5% to form a developer. The distribution of the charge quantity was measured by the toner charge quantity-measuring apparatus shown in Fig. 4. The obtained results are shown in Fig. 1.

By using a remodelled machine (the developing process was changed to the reversal developing process) of Laser Beam Printer LPX-1 (supplied by Mita Industrial Co.) having an organic photosensitive material for negative charging mounted thereon (surface potential of photosensitive material: -700 V, developing bias voltage: - 500 V), the above-mentioned developer was subjected to the continuous copying test for forming 1,000 prints. Reduction of the image density or occurrence of fogging of the image was not observed, and scattering of the toner was not caused.

The obtained results are shown in Table 1.

Furthermore, 50,000 prints were continuously formed and the distribution of the charge quantity was measured. As shown in Fig. 5, the obtained curve of the distribution was substantially as sharp as in intial stage.

### Example 2

A toner having an average particle size of 11 µm was prepared in the same manner as described in Example 1 except that 2 parts by weight of a copolymer (Mw: 10,000) as the charge-controlling agent and 0.5 part by weight of a quaternary ammonium salt represented by the following formula: was used as the charge-controlling assistant.

Then, in the same manner as described in Example 1, a developer was formed and 50,000 prints were continuously formed. As in Example 1, a good image was obtained, and scattering of the toner in the machine was not caused. Furthermore, the distribution of the charge quantity of the toner was as sharp as in Example 1.

### Comparative Example 1

A toner was prepared in the same manner as described in Example 1 except that the charge-controlling assistant was not used. The distribution of the charge quantity of the toner was measured in the same manner as described in Example 1. The obtained results are shown in Fig. 2. Furthermore, 50,000 prints were continuously formed in the same manner as described in Example 1. The image density was unstable and dropping of the image density often occurred. Fogging of the image or scattering of the toner was sometimes caused.

### Comparative Example 2

A toner was prepared in the same manner as described in Example 1 except that 2 parts by weight of Solvent Yellow 56, compatible with the fixing resin, was used instead of the charge-controlling assistant used in Example 1. The distribution of the charge quantity of the toner was measured in the same manner as described in Example 1. The obtained results are shown in Fig. 3. Furthermore, 50,000 prints were continuously formed in the same manner as described in Example 1. Fogging of the image and scattering of the toner were conspicuous. The image density was satisfactory to some extent, but the density often became uneven.

### Comparative Example 3

A toner was prepared in the same manner as described in Example 1 except that 2 parts by weight of a chromium-containing monoazo dye was used instead of the negative charge-controlling agent used in Example 1. The distribution of the charg quantity of the resulting toner is shown in curve A in Fig. 6. In the continuous formation of 5000 points, a good image was obtained in the early times and scattering of the toner was none in the apparatus. But at the end (from 4,500 print soon) small fog density and variation in the density of the image were noted.

The distribution of charg quantity before the formation of continuous image is shown in Fig. 6 curve B a comparison of curve A and B shows that as the image is formed, the distribution of charged amount was broad, and pooly charged toners developed.

### Example 3

A toner (yellow toner) having an average particle size of 11 µm was prepared in the same manner as described in Example 1 by using 100 parts by a styrene/acrylic copolymer as the fixing resin, 5 parts by weight of C.I. Pigment Yellow 17 as the colorant, 1.5 parts by weight of low-molecular-weight polypropylene as the offset-preventing agent, 2 parts by weight of the copolymer used in Example 1 as the charge-controlling agent for negative charging and 0.5 part by weight of the quaternary ammonium salt used in Example 1.

Then, a developer was prepared in the same manner as described in Example 1, and the distribution of the charge quantity was measured by using the apparatus shown in Fig. 4. A sharp distribution shown in curve A in Fig. 7 was observed.

Furthermore, in the same manner as described in Example 1, 50,000 prints were continuously formed and the image characteristics were observed, and the distribution of the charge quantity was measured. A good image having no scattering of the toner was obtained.

The obtained distribution curve (curve B in Fig. 7) was as sharp as the curve A of the initial distribution of the charge quantity.

### Example 4

A toner (yellow toner) was prepared in the same manner as described in Example 3 except that 5 parts by weight of C.I. Pigment Yellow 13 was used as the colorant and 0.5 part by weight of the quaternary ammonium salt used in Example 2 was used as the charge-controlling assistant.

The distribution of the charge quantity was measured in the same manner as described in Example 1. The obtained distribution curve was sharp and similar to the curve A in Fig. 7.

Furthermore, in the same manner as described in Example 3, the image characteristics were observed after 50,000 prints were continuously formed, and the distribution of the charge quantity was measured. Scattering of the toner was not caused and a good image was obtained, and the distribution of the charge quantity was substantially as sharp as in the initial stage.

### Comparative Example 4

A toner was prepared in the same manner as described in Example 3 except that 0.5 part by weight of C.I. Solvent Yellow 56 compatible with the fixing resin was used instead of the charge-controlling assistant used in Example 3. The distribution of the charge quantity of the toner was measured in the same manner as described in Example 1. A board distribution similar to that shown in Fig. 3 was observed.

When 1,000 prints were continuously formed, fogging of the image and scattering of the toner were conspicuous. The image density was satisfactory to some extent, but density unevenness was sometimes caused.

### Example 5

A toner (magenta toner) was prepared in the same manner as described in Example 3 except that 5 parts by weight of C.I. Pigment Red 122 was used as the colorant. A sharp distribution shown in the curve A in Fig. 8 was obtained.

In the same manner as described in Example 3, 50,000 prints were continuously formed and the distribution of
the charge quantity was measured. As shown by the curve B in Fig. 8, the obtained distribution was sharp and was not substantially different from the initial distribution (curve A) of the charge quantity.

### Example 6

A toner (magenta toner) was prepared in the same manner as described in Example 4 except that 5 parts by weight of C.I. Pigment Red 122 was used as the colorant. A sharp distribution similar to that shown in the curve A in Fig. 8 was obtained.

In the same manner as described in Example 4, 50,000 prints were continuously formed and the distribution of the charge quantity was measured. The obtained distribution was sharp and was not substantially different from the initial distribution of the charge quantity.

### Example 7

A toner (cyan toner) was prepared in the same manner as described in Example 3 except that 5 parts by weight of C.I. Pigment Blue 15 was used as the colorant. A sharp distribution similar to that shown in the curve A in Fig. 9 was obtained.

In the same manner as described in Example 3, 50,000 prints were continuously formed and the distribution of the charge quantity was measured. As shown by the curve B in Fig. 9, the obtained distribution was sharp and was not substantially different from the initial distribution (curve A) of the charge quantity.

### Example 8

A toner (cyan toner) was prepared in the same manner as described in Example 4 except that 5 parts by weight of C.I. Pigment Blue 15 was used as the colorant. A sharp distribution similar to that shown in the curve A in Fig. 9 was obtained.

In the same manner as described in Example 4, 50,000 prints were continuously formed and the distribution of the charge quantity was measured. The obtained distribution was sharp and was not substantially different from the initial distribution of the charge quantity.

## Claims

1. An electrophotographic toner for negative charging, comprising a fixing resin, a colorant, a charge controlling agent for negative charging which is a copolymer of an acrylamide monomer of formula (I)
CH₂ = CX¹ - CONH - X² -SO₃H (I)
wherein X¹ is hydrogen or methyl and X² is a divalent
hydrocarbon group having 1 to 6 carbon atoms and a vinylic monomer, and a charge-controlling assistant which is a positive charge-controlling substance which is incompatible with the fixing resin and is dispersed therein and which charge-controlling assistant is a compound of formula (II)
wherein one or two of the groups R are alkyl or alkenyl having at least 8 carbon atoms and the other groups R are alkyl of up to 4 carbon atoms or benzyl and A⁻ is an oxyacid anion.

2. A toner according to claim 1 wherein at least one of the groups R is alkyl or alkenyl of 8 to 22 carbon atoms.

3. A toner according to claim 1 or 2 wherein the charge-controlling assistant is a quaternary ammonium salt of orthophosphoric acid, molybdic acid, tungstic acid, antimonic acid or bismuthic acid.

4. A toner according to any one of claims 1 to 3 wherein the charge-controlling agent and the charge-controlling assistant are present at a weight ratio of from 1:0.05 to 1:1, and are used in a total amount of 0.5 to 5 parts by weight per 100 parts by weight of the fixing resin.

5. A toner according to any one of claims 1 to 4 wherein the charge-controlling agent is a copolymer which contains 2 to 20% by weight of the acrylamide monomer.

6. A toner according to any one of claims 1 to 5 wherein the charge-controlling agent is a copolymer of an acrylamide and styrene.

7. A toner according to claim 6 wherein the charge-controlling agent is a copolymer of 2-acrylamide-2-methylpropanesulphonic acid and styrene.

8. A toner according to claim 7 wherein the copolymer has a weight-average molecular weight (Mw) of 2,000 to 15,000.

9. A yellow toner according to any one of claims 1 to 8 wherein the colorant is a benzidine pigment.

10. A magenta toner according to any one of claims 1 to 8 wherein the colorant is a quinacridone pigment.

11. A cyan toner according to any one of claims 1 to 8 wherein the colorant is a copper-phthalocyanine pigment.

12. Use of a toner according to any one of claims 1 to 11 in electrophotographic printing and electrophotographic reproduction of images.

13. A two-component magnetic developer comprising a toner as claimed in any one of claims 1 to 11 and a magnetic carrier.

14. A process for producing an electrophotographic toner for negative charging which process comprises melt-kneading a mixture comprising comprising a fixing resin, a colorant, a charge controlling agent for negative charging which is a copolymer of an acrylamide monomer of formula (I)
CH₂ = CX¹ - CONH - X² -SO₃H (I)
wherein X¹ is hydrogen or methyl and X² is a divalent
hydrocarbon group having 1 to 6 carbon atoms
and a vinylic monomer, and a charge-controlling assistant which is a positive charge-controlling substance which is incompatible with the fixing resin and is dispersed therein and which charge-controlling assistant is a compound of formula (II)
wherein one or two of the groups R are alkyl or alkenyl having at least 8 carbon atoms and the other groups R are alkyl of up to 4 carbon atoms or benzyl and A⁻ is an oxyacid anion.

15. A process according to claim 14 for producing a toner as defined in any one of claims 2 to 11.

16. A process for producing a two component magnetic developer which process comprises mixing a magnetic carrier with an electrophotographic toner for negative charging, comprising a fixing resin, a colorant, a charge controlling agent for negative charging which is a copolymer of an acrylamide monomer of formula (I)
CH₂ = CX¹ - CONH - X² -SO₃H (I)
wherein X¹ is hydrogen or methyl and X² is a divalent
hydrocarbon group having 1 to 6 carbon atoms
and a vinylic monomer, and a charge-controlling assistant which is a positive charge-controlling substance which is incompatible with the fixing resin and is dispersed therein and which charge-controlling assistant is a compound of formula (II)
wherein one or two of the groups R are alkyl or alkenyl having at least 8 carbon atoms and the other groups R are alkyl of up to 4 carbon atoms or benzyl and A⁻ is an oxyacid anion.

17. A process according to claim 16 wherein the toner is as defined in any one of claims 2 to 11.

## Patentansprüche

1. Elektrophotographischer Toner für negative Aufladung, dadurch gekennzeichnet, daß er ein Fixierharz, ein Farbmittel, ein Ladungskontrollmittel für negative Aufladung, das ein Copolymer eines Acrylamid-Monomers der Formel (I),
CH₂ = CX¹ - CONH - X² -SO₃H (I)
worin X¹ Wasserstoff oder Methyl ist und X² eine zweiwertige Kohlenwasserstoffgruppe mit 1 bis 6 Kohlenstoffatomen bedeutet, und eines Vinyl-Monomers ist, und ein Ladungskontroll-Hilfsmittel, das ein eine positive Ladung kontrollierender Stoff ist, der mit dem Fixierharz inkompatibel und darin dispergiert ist, umfaßt, und worin das Ladungskontroll-Hilfsmittel eine Verbindung der Formel (II) ist worin eine oder zwei der Reste R Alkyl oder Alkenyl mit mindestens 8 Kohlenstoffatomen bedeuten, und die anderen Reste R Alkyl mit bis zu 4 Kohlenstoffatomen oder Benzyl sind, und A⁻ ein Anion einer Sauerstoffsäure ist.

2. Toner nach Anspruch 1, dadurch gekennzeichnet, daß mindestens einer der Reste R Alkyl oder Alkyenyl mit 8 bis 22 Kohlenstoffatomen ist.

3. Toner nach Anspruch 1 oder 2, dadurch gekennzeichnet, daß das Ladungskontroll-Hilfsmittel ein quaternäres Ammoniumsalz einer Orthophosphorsäure, Molybdänsäure, Wolframsäure, Antimonsäure oder Bismutsäure ist.

4. Toner nach einem der Ansprüche 1 bis 3, dadurch gekennzeichnet, daß das Ladungskontrollmittel und das Ladungskontroll-Hilfsmittel in einem Gewichtsverhältnis von 1:0.05 bis 1:1 vorhanden sind, und in einer Gesamtmenge von 0.5 bis 5 Gewichtsteile pro 100 Gewichtsteile des Fixierharzes verwendet werden.

5. Toner nach einem der Ansprüche 1 bis 4, dadurch gekennzeichnet, daß das Ladungskontrollmittel ein Copolymer ist, das 2 bis 20 Gew.-% des Acrylamid-Monomers enthält.

6. Toner nach einem der Ansprüche 1 bis 5, dadurch gekennzeichnet, daß das Ladungskontrollmittel ein Copolymer eines Acrylamids und Styrol ist.

7. Toner nach Anspruch 6, dadurch gekennzeichnet, daß das Ladungskontrollmittel ein Copolymer von 2-Acrylamid-2-methylpropansulfonsäure und Styrol ist.

8. Toner nach Anspruch 7, dadurch gekennzeichnet, daß das Copolymer ein mittleres Molekulargewicht (Mw) von 2000 bis 15000 besitzt.

9. Gelbtoner nach einem der Ansprüche 1 bis 8, dadurch gekennzeichnet, daß das Farbmittel ein Benzidinpigment ist.

10. Magentatoner nach einem der Ansprüche 1 bis 8, dadurch gekennzeichnet, daß das Farbmittel ein Chinacridonpigment ist.

11. Cyantoner nach einem der Ansprüche 1 bis 8, dadurch gekennzeichnet, daß das Farbmittel ein Kupferphthalocyaninpigment ist.

12. Verwendung eines Toner nach einem der Ansprüche 1 bis 11 in elektrophotographischen Druckverfahren und elektrophotographischen Reproduktionsverfahren von Bildern.

13. Magnetischer Zweikomponenten-Entwickler, dadurch gekennzeichnet, daß er einen Toner nach einem der Ansprüche 1 bis 11 und einen Magnetträger enthält.

14. Verfahren zur Herstellung eines elektrophotographischen Toners für negative Aufladung, dadurch gekennzeichnet, daß das Verfahren umfaßt: Schmelzkneten einer Mischung umfassend ein Fixierharz, ein Farbmittel, ein Ladungskontrollmittel für negative Aufladung, das ein Copolymer eines Acrylamid-Monomers der Formel (I)
CH₂ = CX¹ - CONH - X² -SO₃H (I)
worin X¹ Wasserstoff oder Methyl und X² eine zweiwertige Kohlenwasserstoffgruppe mit 1 bis 6 Kohlenstoffatomen bedeutet, und eines Vinyl-Monomers ist, und ein Ladungskontroll-Hilfsmittel, das ein eine positive Ladung kontrollierender Stoff ist, der mit dem Fixierharz inkompatibel und darin dispergiert ist, und worin das Ladungskontrollmittel eine Verbindung der Formel (II) ist worin eine oder zwei der Reste R Alkyl oder Alkenyl mit mindestens 8 Kohlenstoffatomen bedeuten und die anderen Reste R Alkyl mit bis zu 4 Kohlenstoffatomen oder Benzyl sind, und A⁻ ein Anion einer Sauerstoffsäure ist.

15. Verfahren nach Anspruch 14 zur Herstellung eines Toners gemäß einem der Ansprüche 2 bis 11.

16. Verfahren zur Herstellung eines magnetischen Zweikomponenten-Entwicklers, dadurch gekennzeichnet, daß das Verfahren umfaßt: Mischen eines Magnetträgers mit einem elektrophotographischen Toner für negative Aufladung, der ein Fixierharz, ein Farbmittel, ein Ladungskontrollmittel für negative Aufladung, das ein Copolymer eines Acryl-Monomers der Formel (I)
CH₂ = CX¹ - CONH - X² -SO₃H (I)
worin X¹ Wasserstoff oder Methyl ist und X² eine zweiwertige Kohlenwasserstoffgruppe mit 1 bis 6 Kohlenstoffatomen bedeutet, und einem Vinyl-Monomer ist, und ein Ladungskontroll-Hilfsmittel, das ein eine positive Ladung kontrollierender Stoff ist, der mit dem Fixierharz inkompatibel und darin dispergiert ist, umfaßt, und worin das Ladungskontroll-Hilfsmittel eine Verbindung der Formel (II) ist worin eine oder zwei der Reste R Alkyl oder Alkenyl mit mindestens 8 Kohlenstoffatomen bedeuten und die anderen Reste R Alkyl mit bis zu 4 Kohlenstoffatomen oder Benzyl sind, und A⁻ ein Anion einer Sauerstoffsäure ist.

17. Verfahren nach Anspruch 16, dadurch gekennzeichnet, daß der Toner ein solcher gemäß einem der Ansprüche 2 bis 11 ist.

## Revendications

1. Toner électrophotographique pour charger négativement, comprenant une résine de fixage, un colorant, un agent de contrôle de charge pour charger négativement qui est un copolymère d'un monomère d'acrylamide de formule (I) :
CH₂ = CX¹ - CONH - X² - SO₃H (I)
dans laquelle X¹ est un atome d'hydrogène ou un groupe méthyle et X² est un groupe hydrocarbure divalent ayant 1 à 6 atomes de carbone
et d'un monomère vinylique, et une aide au contrôle de charge qui est une substance de contrôle de charge positive incompatible avec la résine de fixage et y dispersée, aide au contrôle de charge qui est un composé de la formule (II) : dans laquelle un ou deux des groupes R sont un groupe alkyle ou alcényle ayant au moins 8 atomes de carbone et les autres groupes R sont un groupe alkyle ayant jusqu'à 4 atomes de carbone ou un groupe benzyle et A⁻ est un anion d'oxyacide.

2. Toner selon la revendication 1, dans lequel au moins l'un des groupes R est un groupe alkyle ou alcényle ayant 8 à 22 atomes de carbone.

3. Toner selon la revendication 1 ou 2, dans lequel l'aide au contrôle de charge est un sel d'ammonium quaternaire d'un acide orthophosphorique, acide molybdique, acide tungstique, acide antimonique ou acide bismuthique.

4. Toner selon l'une quelconque des revendications 1 à 3, dans lequel l'agent de contrôle de charge et l'aide au contrôle de charge sont présents suivant un rapport pondéral de 1:0,05 à 1:1, et sont utilisés dans une quantité totale de 0,5 à 5 parties en poids pour 100 parties en poids de la résine de fixage.

5. Toner selon l'une quelconque des revendications 1 à 4, dans lequel l'agent de contrôle de charge est un copolymère qui contient 2 à 20 % en poids du monomère d'acrylamide.

6. Toner selon l'une quelconque des revendications 1 à 5, dans lequel l'agent de contrôle de charge est un copolymère d'un acrylamide et de styrène.

7. Toner selon la revendication 6, dans lequel l'agent de contrôle de charge est un copolymère de l'acide 2-acrylamide-2-méthylpropane-sulfonique et de styrène.

8. Toner selon la revendication 7 dans lequel le copolymère a une masse moléculaire moyenne en masse (Mw) de 2 000 à 15 000.

9. Toner jaune selon l'une quelconque des revendications 1 à 8, dans lequel le colorant est un pigment de benzidine.

10. Toner magenta selon l'une quelconque des revendications 1 à 8, dans lequel le colorant est un pigment de quinacridone.

11. Toner cyan selon l'une quelconque des revendications 1 à 8, dans lequel le colorant est un pigment de cuivre-phtalocyanine.

12. Utilisation d'un toner selon l'une quelconque des revendications 1 à 11 dans l'impression électrophotographique et la reproduction électrophotographique d'images.

13. Révélateur magnétique à deux composants comprenant un toner tel que revendiqué dans l'une quelconque des revendications 1 à 11 et un support magnétique.

14. Procédé pour préparer un toner électrophotographique pour charger négativemnt, procédé qui comprend le malaxage en masse fondue d'un mélange comportant une résine de fixage, un colorant, un agent de contrôle de charge pour charger négativement qui est un copolymère d'un monomère d'acrylamide de formule (I):
CH₂ = CX¹ - CONH - X² -SO₃H (I)
dans laquelle X¹ est un atome d'hydrogène ou un groupe méthyle et X² est un groupe hydrocarbure divalent ayant 1 à 6 atomes de carbone
et d'un monomère vinylique, et une aide au contrôle de charge qui est une substance de contrôle de charge positive incompatible avec la résine de fixage et y est dispersée, aide au contrôle de charge qui est un composé de la formule (II) : dans laquelle un ou deux des groupes R sont un groupe alkyle ou alcényle ayant au moins 8 atomes de carbone et les autres groupes R sont un groupe alkyle ayant jusqu'à 4 atomes de carbone ou un groupe benzyle et A⁻ est un anion d'oxyacide.

15. Procédé selon la revendication 14 pour la préparation d'un toner tel que défini dans l'une quelconque des revendications 2 à 11.

16. Procédé pour préparer un révélateur magnétique à deux composants, procédé qui comprend le mélange d'un support magnétique avec un toner électrophotographique pour charger négativement, comportant une résine de fixage, un colorant, un agent de contrôle de charge pour charger négativement qui est un copolymère d'un monomère d'acrylamide de formule (I):
CH₂ = CX¹ - CONH - X² -SO₃H (I)
dans laquelle X¹ est un atome d'hydrogène ou un groupe méthyle et X² est un groupe hydrocarbure divalent ayant 1 à 6 atomes de carbone
et d'un monomère vinylique, et une aide au contrôle de charge qui est une substance de contrôle de charge positive qui est incompatible avec la résine de fixage et y dispersée, aide au contrôle de charge qui est un composé de la formule (II) : dans laquelle un ou deux des groupes R sont un groupe alkyle ou alcényle ayant au moins 8 atomes de carbone et les autres groupes R sont un groupe alkyle ayant jusqu'à 4 atomes de carbone ou un groupe benzyle et A⁻ est un anion d'oxyacide.

17. Procédé selon la revendication 16, dans lequel le toner est tel que défini dans l'une quelconque des revendications 2 à 11.
